

April 6, 1948.

E. L. COE

2,439,039

PROCESS OF PRODUCING MEDULLATED ARTIFICIAL FILAMENTS

Filed Sept. 26, 1944



*Fig. 1*



*Fig. 4*



*Fig. 2*



*Fig. 3*

*Elvin L. Coe*  
INVENTOR.

*BY Carl A. Castellan*  
attorney

## UNITED STATES PATENT OFFICE

2,439,039

PROCESS OF PRODUCING MEDULLATED  
ARTIFICIAL FILAMENTSElvin L. Coe, Nitro, W. Va., assignor to American  
Viscose Corporation, Wilmington, Del., a cor-  
poration of Delaware

Application September 26, 1944, Serial No. 555,809

4 Claims. (Cl. 18—54)

1

This invention relates to methods of producing wool-like medullated artificial filaments and fibers. More specifically, the invention relates to methods of producing wool-like medullated artificial filaments and fibers from viscose.

Previously, in order to produce medullated artificial filaments or fibers from viscose, it has been considered necessary to utilize viscose which had been ripened considerably beyond the age of viscose conventionally used for the manufacture of artificial filaments and fibers. The filaments and fibers obtained from such over-aged or over-ripened viscose were characterized by extremely low wet and dry tensile strengths. It was also suggested, in one instance, to produce such artificial filaments and fibers by spinning a viscose of extremely high viscosity, prepared by immediately xanthating unaged alkali cellulose, into a spinning bath containing abnormally high amounts of zinc sulfate.

When viscose is extruded through a suitable spinneret or jet into a coagulating and regenerating bath, there is formed, first, a thin outer tube of regenerated cellulose, enclosing a core of fluid viscose, which fluid viscose is coagulated and regenerated subsequently by diffusion of the bath through the first-formed outer skin.

The present invention is based upon the discovery that it is possible to adjust the electrolytic concentrations of the fluid viscose core and the spinning bath, which affects the rate of diffusion of the bath through the outer skin, and thus makes it possible to control and retard the diffusion rate, so that the membranous outer skin may be uniformly ruptured or cracked, by means of stretching, while the inner core of viscose which it encloses is still in the fluid state. According to my invention, such diffusion control is achieved by incorporating a soluble salt, notably sodium sulfate, with the viscose at any point prior to extrusion of the latter into the spinning bath, and extruding the viscose into a spinning bath containing controlled amounts of sulfuric acid and zinc sulfate.

Generally speaking, there is used in accordance with the present invention any normal viscose which is suitable for spinning artificial filaments according to the conventional methods, that is a viscose having a common salt (sodium chloride) point of from about 2.7 to 4.1. However, it is preferred to use a viscose having a cellulose content in the neighborhood of about 8% and containing sodium hydroxide in relatively high concentration. The sodium hydroxide content of the viscose however, is lower than

2

the cellulose content, for best results. The viscose may contain special modifying agents such as dulling agents, dyes, or pigments, or mixtures of such materials according to this invention.

5 The sodium sulfate may be added to the viscose in any amount, but it is preferred to use concentrations in the range of from about 2% to 10%, based upon the weight of the viscose, optimum results being usually obtained when the sodium sulfate is present in the viscose in a concentration of about 6 to 8%.

When proceeding according to this invention, viscose containing sodium sulfate is extruded into an aqueous coagulating and regenerating bath 15 containing sodium sulfate and carefully controlled amounts of sulfuric acid, the latter being present in an amount of from 8 to 12%.

The bath may also contain up to 1.25% of zinc sulfate. I have found that, other conditions being as stated previously herein, the appearance 20 of the filaments in cross-section can be predetermined, depending upon whether zinc sulfate is omitted from the spinning bath or present therein in controlled quantities. Thus, if zinc sulfate is omitted, or is present in an amount up to about 0.5%, the filaments obtained have, in cross-section, and along a predominant portion of the filament length, the shape of a horse-shoe the ends of which are comparatively widely 25 spaced apart, whereas when zinc sulfate is present in the bath in amounts ranging from about 0.5 to about 1.25%, the filaments have, in cross-section, and along a predominant portion of the filament length, the configuration of a horse-shoe the ends of which are substantially closed, or in some cases, even overlapped. I have found 30 that whereas when the proportionate relationship of the bath constituents is carefully adjusted as indicated wool-like distinctly medullated filaments are obtained, if the bath contains sulfuric acid in an amount less than 8% or greater than 12%, and zinc sulfate in an amount in excess of 1.25%, medullated filaments cannot be obtained. The useful quantity of sodium sulfate is not so critical and it may be present in varying amounts. Preferably, the sodium sulfate is used in amounts ranging from 21 to 27%.

The preferred conditions for obtaining medullated filaments according to this invention involve the addition of from 6 to 7% of sodium sulfate to a viscose having a common salt (NaCl) point of 3.2 to 3.6 and having about 8% cellulose and about 6.6% sodium hydroxide (based on the weight of the viscose), and extrusion of such viscose into an aqueous spinning bath containing

from 8 to 12% sulfuric acid, about 1% zinc sulfate, and from 21 to 27% sodium sulfate.

The spinning bath is preferably maintained at a temperature of about 45 to 50° C.

After suitable immersion in the special coagulating and regenerating bath, the extruded filaments are withdrawn and subjected to stretching. The length of immersion of the filaments in the bath, and the degree of stretch given them are important factors in achieving both rupturing or cracking of the outer membranous tube of regenerated cellulose, and medullation. The length of immersion of the filaments in the coagulating and regenerating bath may be varied somewhat but, in general, it is observed that best results are obtained with relatively short immersion distances, say in the neighborhood of about 14 to 30". Of course, a wider range of limits may be used, depending upon the spinning speeds employed. The coagulation and regeneration is preferably effected under relaxed conditions, that is, the velocity of the filaments as they are drawn from the bath is maintained lower than the velocity of extrusion. After withdrawal from the bath, the filaments may be subjected to stretching up to about 50% of their length, but preferably a lower degree of stretching, on the order of about 15 to 20%, is used.

This invention will be more readily understood by reference to the accompanying drawing, in which

Figure 1 is a side view, greatly enlarged, of a filament produced according to my invention;

Figure 2 is a greatly enlarged end view of one type of filaments obtained according to the invention;

Figure 3 is a greatly enlarged end view of another type of filaments obtained according to the invention; and

Figure 4 is a diagrammatic view of a spinning device which may be used for spinning artificial wool-like filaments in accordance with the present invention.

Referring to Figure 4, the viscose containing from 2 to 10% sodium sulfate is extruded through the orifices of spinneret 1 into an aqueous coagulating and regenerating bath 2 having the composition set forth above and maintained at about 45 to 50° C.

The filaments are drawn from the bath and passed over a godet 3, and then over a second godet 4, the latter rotating at a peripheral speed greater than the speed of godet 3. The filaments are stretched between the godets. Stretching may be effected by any customary or known means, and, if desired, godet 4 may be replaced by a tow-roll which receives filaments from a number of spinnerets.

The filaments may then be directed to a suitable wind-up device, such as the centrifuge 5, shown in Figure 4, or, if it is desired to cut them to staple fiber length, they are directed to the mouth of a cutting device, where they are cut, in the wet state, and then dried. During drying the fibers tend to spiral and that, together with the preferred relaxed spinning conditions, appears to insure a permanent and natural crimp therein.

The filaments may be subjected to the usual after-treatments, such as desulphurizing, etc., before collection or cutting to staple lengths. Alternatively, they may be after-processed after collection or after cutting to staple fibers.

The artificial wool-like filaments and fibers produced according to this invention are medul-

lated, that is, they have, in cross-section, a horse-shoe shape apparently caused by the filaments first forming a ribbon, and then folding in such a manner as to form a hollow tube with a slit on one side. The tube-like structure thus has a hollow, air-enclosing space or canal in the center thereof, providing occluded air spaces, which impart to the filaments or fibers insulating properties similar to those of natural wool. The products are characterized by a curled, kinky, or crimped form, which is assumed spontaneously and which persists as one of their permanent structural characteristics. Because they are stretched while the inner core of viscose is still in relatively fluid condition the surface of the filaments has a series of substantially uniform transverse and longitudinal cracks, as shown at 6 and 7, in Figure 1, which impart a roughness to the surface which is similar to, and has the same effect, particularly during textile processing, as the epidermal scales of natural wool fibers. The products of this invention are further characterized by a subdued luster or matt-like appearance, which is natural, and which is obtained without the addition to the viscose of any foreign delustering agents, such as pigments, oils, or the like, although, of course, if desired, such foreign delustering agents may be utilized.

The fibers differ from standard rayon staple fiber in their increased power to absorb water, and in their different dye index, the fibers obtained by the present invention having a more pronounced ability to absorb dye, and being capable of being dyed darker and deeper than standard staple fibers, treated in the same dye bath.

The products of this invention are suitable for a wide variety of uses.

Because of their medullated form, they possess good insulating properties and, due to their roughened or scale-like surface and natural crimp, they show good cohesion or coherence in textile operations, where they may be precessed, either alone or admixed in blends with other fibers.

The products may be utilized in the form of continuous filaments, or cut into staple of any desired length. Either alone or in admixture with wool, crimped rayon staple, standard staple, or the like, they may be converted into yarns by conventional procedures, as by spinning in accordance with the cotton, woolen, worsted, or modified systems. Fabrics composed of such yarns possess unusual properties as to "hand" or "feel."

The medullated artificial wool-like filaments produced according to my invention have been found to have tensile strengths of at least about 1 to 1½ gms./denier, and extensibilities of at least 10% to 25% when dry; and to have tensile strengths of at least about ½ to 1 gms./denier, and extensibilities of at least 10 to 40% when wet.

The following examples illustrate methods of producing artificial medullated wool-like filaments and fibers according to my invention.

#### Example I

A viscose having 8% cellulose, 6.6% sodium hydroxide (based on the weight of the viscose), aged to a salt point of 3.5, and having a ball fall viscosity of 65 sec. and to which was added 8% of sodium sulfate (based on the weight of the viscose), was extruded to form filaments of 7.5 denier through a spinneret having holes 2.5 mils

## 5

in diameter, into an aqueous coagulating and regenerating bath containing.

|                | Per cent |
|----------------|----------|
| Sulfuric acid  | 10.5     |
| Sodium sulfate | 21       |
| Zinc sulfate   | 1        |

at a temperature of 45° C. The filaments were immersed in the bath for a distance of 30 inches, and then gathered around a driven glass wheel. From the glass wheel, the filaments were passed to a tow-roll driven at a linear speed of 52 meters a minute, and given a 15% stretch between the wheel and tow-roll. The medullated filaments upon leaving the tow-roll were directed to a cutting device and, after cutting, the fibers were opened and then dried. The fibers developed a permanent natural crimp during the drying procedure and were medullated.

## Example II

A viscose having 8% cellulose, 6% sodium hydroxide (based on the weight of the viscose) which was aged to a salt point of 3.6, and to which had been added 7.3% sodium sulfate (based on the weight of the viscose) was extruded to form filaments of 5.5 denier, through a spinneret having holes 2.5 mils in diameter, into a coagulating and regenerating bath as described in Example I. The filaments were immersed in the bath for a distance of 14 inches, stretched as described in Example I, and the filaments, which were distinctly medullated in character, were then directed to a wind-up device. The filaments had, in cross-section, and along a preponderant portion of their length, a substantially closed horseshoe shape as shown in Figure 2.

## Example III

A viscose having 8% cellulose, 6.4% sodium hydroxide (based on the weight of the viscose), which was aged to a salt point of 3.6, and to which had been added 6.7% of sodium sulfate (based on the weight of the viscose) was extruded to form filaments of 5.5 denier through a spinneret having holes 2.5 mils in diameter, into a coagulating and regenerating bath as described in Example I. The filaments were immersed in the bath for a distance of 14 inches, and then handled as described in Example I. The products were medullated.

## Example IV

A viscose having 8% cellulose, 7% sodium hydroxide (based on the weight of the viscose) which was aged to a salt point of 3.2, and to which had been added 6.5% of sodium sulfate (based on the weight of the viscose) was extruded to filaments of 5.5 denier through a spinneret having holes 2.5 mils in diameter, into an aqueous coagulating and regenerating bath containing

|                | Per cent |
|----------------|----------|
| Sulfuric acid  | 8.5      |
| Sodium sulfate | 21       |
| Zinc sulfate   | 1        |

at a temperature of 50° C. The filaments were immersed in the bath for a distance of 19 inches, and then handled as described in Example I. The fibers thus obtained were medullated.

## Example V

A viscose having 8% cellulose, 6.6% sodium hydroxide (based on the weight of the viscose) which was aged to a salt point of 4.0 and to which had been added 6.0% of sodium sulfate

(based on the weight of the viscose) was extruded to filaments of 5.5 denier through a spinneret having holes 2.5 mils in diameter, into an aqueous coagulating and regenerating bath containing

|                | Per cent |
|----------------|----------|
| Sodium sulfate | 27       |
| Sulfuric acid  | 11.5     |
| Zinc sulfate   | 1        |

at a temperature of 45° C. The filaments were immersed in the bath for a distance of 14 inches, and then handled as described in Example I. The products thus obtained were medullated.

## Example VI

A viscose having 7.5% cellulose, 6% sodium hydroxide (based on the weight of the viscose) which was aged to a salt point of 3.6, and to which had been added 7% of sodium sulfate (based on the weight of the viscose) was extruded to filaments of 5.5 denier through a spinneret having holes 2.5 mils in diameter, into an aqueous coagulating and regenerating bath containing

|                | Per cent |
|----------------|----------|
| Sulfuric acid  | 9.5      |
| Sodium sulfate | 27.0     |
| Zinc sulfate   | 1.25     |

at a temperature of 50° C. The filaments were immersed in the bath for a distance of 14 inches, and then gathered around a driven glass wheel. From the glass wheel, the filaments were passed to a tow-roll driven at linear speed of 52.0 M./minute. Between the wheel and tow-roll, the filaments were treated with hot water (90° C.) and given a stretch of 15%. The medullated filaments upon leaving the tow-roll were directed to a cutting device, and handled as described in Example I.

## Example VII

A viscose having 8% cellulose, 6.6% sodium hydroxide (based on the weight of the viscose) which was aged to a common salt (NaCl) point of 2.7, and to which had been added 5% of sodium sulfate (based on the weight of the viscose), was extruded into an aqueous coagulating and regenerating bath containing

|                | Percent |
|----------------|---------|
| Sulfuric acid  | 8       |
| Sodium sulfate | 21      |
| Zinc sulfate   | 0.5     |

at a temperature of 45° C. The distinctly medullated filaments were handled in the manner described above. The filaments so obtained had, in cross-section, and along a preponderant portion of their length, a substantially open horseshoe shape, as shown in Figure 3.

Since it will be apparent that the methods specifically illustrated in the foregoing examples are capable of some modification without departing from the spirit of this invention, it is to be understood that the invention is not to be limited except as set forth in the appended claims.

This application is a continuation-in-part of my prior application, Serial No. 512,890, filed December 4, 1943, now abandoned.

In the claims, where the term "fibers" is used, it is intended to define both continuous filaments and discontinuous fibers.

I claim:

1. A process for the production of artificial fibers having, in cross section, a horseshoe shape comprising the steps of spinning a normal viscose

of normal spinning viscosity, having a salt point of from 2.7 to 4.1 and containing sodium sulphate into a coagulating and regenerating bath consisting of an aqueous solution of sulphuric acid in a concentration of from 8 to 12%, 21 to 27% sodium sulphate, and from 0 to not more than 1.25% of zinc sulphate.

2. A process for the production of artificial fibers having, in cross section, a horseshoe shape comprising the steps of spinning a normal viscose of normal spinning viscosity having a salt point of from 2.7 to 4.1 and containing between 2 and 10% of sodium sulphate based on the weight of the viscose, into a coagulating and regenerating bath consisting of an aqueous solution of sulphuric acid in a concentration of from 8 to 12%, 21 to 27% sodium sulphate, and from 0 to not more than 1.25% of zinc sulphate.

3. A process for the production of artificial fibers having, in cross section, a horseshoe shape comprising the steps of spinning a normal viscose of normal spinning viscosity having a salt point of from 2.7 to 4.1 and containing between 2 and 10% of sodium sulphate based on the weight of the viscose into a coagulating and regenerating bath consisting of an aqueous solution of sulphuric acid in a concentration of from 8 to 12%, 21 to 27% sodium sulphate and from 0 to not more than 0.5% of zinc sulphate.

4. A process for the production of artificial fibers having, in cross section, a horseshoe shape comprising the steps of spinning a normal viscose of normal spinning viscosity having a salt point of from 2.7 to 4.1 and containing between 2 and 10% of sodium sulphate based on the weight of the viscose, spinning the mixture into a coagulating and regenerating bath consisting of an aqueous solution of sulphuric acid in a concentration of from 8 to 12%, 21 to 27% sodium sulphate, and from 0.05 to not more than 1.25% of zinc sulphate.

ELVIN L. COE.

#### REFERENCES CITED

The following references are of record in the file of this patent:

#### UNITED STATES PATENTS

| Number    | Name       | Date          |
|-----------|------------|---------------|
| 1,683,199 | Lilienfeld | Sept. 4, 1928 |
| 2,302,077 | Kohorn     | Nov. 17, 1942 |

#### FOREIGN PATENTS

| Number  | Country       | Date          |
|---------|---------------|---------------|
| 298,548 | Great Britain | Oct. 8, 1928  |
| 339,050 | Germany       | July 12, 1921 |
| 342,641 | Germany       | Oct. 21, 1921 |